

## UNITED STATES PATENT OFFICE

2,159,013

TEXTILE AND OTHER MATERIALS AND  
PROCESS FOR THEIR PRODUCTION

Henry Dreyfus, London, England

No Drawing. Application March 28, 1936, Serial  
No. 71,457. In Great Britain April 9, 1935

6 Claims. (Cl. 8—129)

This invention relates to improved textile and other materials and process for their production.

Commercial cellulose acetate artificial silk is readily delustrated by hot or boiling water or other aqueous liquors or by moist steam. This process forms the basis of a commercial production of delustrated artificial silks, the common commercial process being to treat the artificial silk in a boiling soap solution for upwards of half an hour. The 10 degree of lustre remaining on the material depends upon the temperature and time of treatment, so that various degrees of lustre are obtainable from a completely matt appearance to a lustre little short of that of the artificial silk as 15 spun.

Similarly, artificial silks made from other organic derivatives of cellulose, for instance cellulose propionate and methyl or ethyl cellulose, are delustrable by means of hot or boiling aqueous 20 liquors or moist steam.

The low lustre of the cellulose acetate artificial silk or of similar artificial silks produced by these processes is, however, not permanent to various treatments to which the materials are commonly 25 subjected either in subsequent processes of manufacture or in laundering operations. In particular the lustre is more or less restored by ironing the materials in a wet condition. The present invention has as its object to render the delustrating produced by hot or boiling aqueous liquors or moist steam resistant to ironing and to other treatments.

I have found that an acetone-soluble cellulose acetate artificial silk which has been delustrated 30 may be subjected to a process of acetylation so as to increase its acetyl content while substantially retaining the low lustre of the artificial silk, and further that the treatment renders the lustre progressively resistant to change by ironing wet. 40 At the same time, depending upon the degree of acetylation, the resistance of the material to heat treatments is increased so that the product of the present invention may be ironed without damage at higher temperatures than are customary in 45 ironing ordinary cellulose acetate artificial silk.

Again according to the degree of acetylation, the resulting material is more or less resistant to further delustring by hot or boiling aqueous liquors and, in addition, its affinity for dyestuffs, 50 and in particular for the dispersed insoluble dyestuffs now customarily applied to cellulose acetate artificial silk, is modified.

The same effect may be produced by esterifying the acetone-soluble cellulose acetate artificial silk 55 with esterifying agents other than acetic an-

hydride, and in a similar way the delustre produced in either artificial silks of organic derivatives of cellulose by hot aqueous treatments may be rendered resistant to ironing by acetylation or other esterification.

The acetylation or other esterification is preferably effected with the aid of an acid anhydride, for example acetic anhydride, propionic anhydride, etc. The anhydrides are, in the pure state, solvents for the artificial silks to be treated and, 10 in order to prevent solution or even incipient solution, must be diluted with appropriate agents which repress the solvent power of the anhydrides. In order to obtain the effect of the present invention, the degree of dilution must be such that 15 the original lustre of the artificial silk is not restored by the acetylation or other esterification, and is preferably such that there is little or no change in the lustre. By this means, the final lustre in the artificial silk may be predetermined by an adjustment of the temperature and time of treatment in the hot aqueous media, and this degree of delustre remains in the after-treatment.

Generally, hydrocarbons and the non-solvent 25 chlorinated hydrocarbons are the most suitable diluents for the purpose of the present invention, for example benzene, toluene, xylene and the higher homologues of benzene, kerosene and other higher boiling petroleum hydrocarbons, carbon tetrachloride and the like. The higher aliphatic ethers are also useful as diluents. Dilution of acetic anhydride with some twenty times its weight of xylene or other aromatic hydrocarbon or chlorinated hydrocarbon is sufficient to 30 prevent any substantial change in the lustre when the acetylation is carried out at the boiling point of the mixture. The invention is not, however, limited to such proportions and the amount of diluent may be any quantity, such as five or ten times up to twenty times or more the quantity of the anhydride, which will prevent restoration of the lustre of the artificial silk, and is preferably such that there is no substantial change in the lustre. The best proportions to use depend partly 35 on the nature of the anhydride and of the diluent and on the temperature of treatment.

The reaction is preferably effected in the presence of a suitable catalyst which may be any of the ordinary catalysts used in the acetylation 45 of cellulose, but in order to increase the heat resistance of the materials it is preferable not to use sulphuric acid, phosphoric acid, and other di- or poly-basic acid catalysts or derivatives thereof which tend to combine with cellulose in 50

an acetylation process. The most useful catalysts are ferric chloride, zinc chloride, stannic chloride and other metal chlorides which have an acid reaction with or without hydrochloric acid, and also the corresponding bromides of these metals with or without hydrobromic acid. Similarly, sodium or potassium acetate or other weakly alkaline salt, preferably corresponding to the acid anhydride being used, may be employed. Mono-basic acids, such as perchloric acid or hydrochloric acid, or other hydrohalide acid may be employed, though they are not so useful as the halide catalysts already mentioned. The catalyst may be dissolved in the reaction mixture or may be applied to the artificial silk before immersion in the reaction mixture. For example, the artificial silk may be treated with an aqueous or other solution of sodium or potassium acetate, and the catalyst dried out in the material before immersion in the acetylation mixture.

As previously indicated, the effect obtained is to some extent dependent upon the degree of esterification or further esterification brought about in the process of the invention. Generally the degree of esterification may be adjusted by using the appropriate amount of acetylating or other esterifying agent and/or by an adjustment of the temperature or time of treatment. In the case of acetylating delusted cellulose acetate artificial silk, a treatment at the boil for half an hour with a mixture containing a quantity of acetic anhydride equal to 1-2 times the weight of the artificial silk under treatment diluted with an amount of xylene or other hydrocarbon equal to 20 times the weight of the acetic anhydride, is sufficient to render the delustre entirely immune to relustring on subsequent ironing in a wet condition. In this treatment, sodium acetate is either present in the reaction mixture or the material is previously impregnated therewith, for example by soaking in a saturated solution of sodium acetate in the cold, centrifuging and drying.

The treatment according to the present invention may be applied to the artificial silk in any suitable form, for example to yarn in the form of hanks or in the form of open wound packages through which the reaction mixture is pumped or sucked, or in the form of woven, knitted or other fabrics. A previous impregnation with the catalyst may be carried out continuously with the acetylation or other esterification. By carrying out the reaction under a pressure in excess of atmospheric pressure, the reaction temperature may be raised above the boiling point of the anhydride or of the diluent, and in consequence shorter times of treatment may be used.

In addition to rendering the more or less low lustre of artificial silk more resistant to wet ironing for example, the treatment of the present invention improves the resistance of the material to heat generally, so that dry ironing may be carried out at a higher temperature, and also modifies the affinity of the materials for dyestuffs. Thus, materials treated in accordance with the invention may be associated in doubled yarns, cords or similar materials or in fabrics, with untreated materials, so as to obtain a mixed textile material which, while exhibiting as a whole an affinity for certain types of dyestuff, for instance the dispersed insoluble colours, is nevertheless capable of being dyed in different shades by immersion in a dye bath containing a single dyestuff, owing to the differential affinities of the different materials constituting the goods. Further colour ef-

fects may be obtained by associating the products of the present invention, with or without artificial silks of cellulose derivatives which have not been treated, with other types of materials, such as cotton, the regenerated cellulose type of artificial silk, or animal fibres.

Local effects may be produced according to the present invention by the local application of the reagents. For example, a fabric may be printed in a design with a wax or other suitable resist, the unprinted portion delusted by treatment of the fabric in a boiling soap solution, the wax or other resist removed, and the whole fabric acetylated. By this means a lustrous pattern on a delusted ground is obtained. If the acetylation or other esterification mixture is suitable, the resist may be removed on immersion of the material in the reaction mixture.

While the invention has been described above more particularly with reference to the treatment of textile materials, it may also be applied to the treatment of films, foils and similar materials of cellulose derivatives where a permanent delusted appearance is desired. For instance, a translucent wrapping foil may be produced by the present invention which does not become transparent when sealing is effected by means of heat treatment.

The products of the present invention are novel. As compared with ordinary bright artificial silk, they present a dull lustre and have, under a lens, the crazed appearance characteristic of cellulose acetate artificial silk which has been delusted by means of boiling water or moist steam, and, at the same time, they are differentiated from this known delusted product by being resistant to relustring on ironing wet.

The following examples illustrate the invention but are not to be considered as limiting it in any way:

#### Example 1

A cellulose acetate artificial silk fabric is delusted by boiling in a 0.25% soap solution at the boil for  $\frac{1}{2}$ -1 hour, depending on the degree of delustre required. The fabric is then treated for about 1 hour at 20-25° C. in a solution containing, per 100 parts of fabric, 150 parts of acetic anhydride, 2000-3000 parts of benzene, and 3 parts of crystallised ferric chloride. The fabric after treatment is removed, washed first with benzene, then with water and dilute alkali to remove traces of acid, and finely dried.

#### Example 2

A fabric, delusted as in Example 1, is acetylated as described in Example 1, but using instead of 3 parts of crystallised ferric chloride a catalyst comprising 1 part of crystallised ferric chloride and 2 parts of hydrogen chloride. The treatment is otherwise the same.

#### Example 3

A fabric, delusted as in Example 1, is treated for about  $\frac{1}{4}$  hour at 20-25° C. in a bath containing, per 100 parts of fabric, 200-300 parts of acetic anhydride, 1000-1500 parts of benzene, 10 parts of zinc chloride and 4 parts of hydrogen chloride. The fabric is then removed, washed first with benzene then with water, and finally dried.

#### Example 4

A fabric, delusted as described in Example 1, is impregnated with a solution containing 35-40% of sodium acetate, and is then centrifuged and

dried. The fabric is then immersed in a bath containing, per 100 parts of fabric, 3000 parts of xylene and 150 parts of acetic anhydride, and is treated at the boiling point for  $\frac{1}{2}$  hour. The 5 fabric is then removed, washed in xylene, dried, washed in water, and finally dried.

*Example 5*

A cellulose acetate artificial silk fabric is printed in any suitable design with molten resin or colophony. The print is cooled to allow the resin to solidify, and the fabric is then treated in water at 90-95° C. until the desired degree of deluster is produced. The fabric is then rinsed and the resin 10 removed, for example by treatment with xylene or other suitable solvent. The fabric is then acetylated according to any of the preceding examples.

The products of Examples 1-4 are all delustered fabrics which present the crazed appearance 20 characteristic of ordinary delustered cellulose acetate artificial silk, but are all resistant to relustering on ironing wet. Further, the treatment has raised the resistance of the fabric to heat. The product of Example 5 is also more resistant 25 to heat than the starting material, but the permanent deluster is in a design on a lustrous background. In a similar way, delustered cellulose acetate artificial silk or delustered cellulose acetate foil may be treated with other esterifying agents; 30 for example propionic or butyric anhydride, and, further, delustered material of other organic derivatives of cellulose may be acetylated or otherwise esterified.

Having described my invention, what I desire to 35 secure by Letters Patent is:

1. Process for the production of artificial materials of reduced luster which is not increased by ironing while wet, which comprises reducing the luster of textile materials, foils, films and 40 similar materials made of organic substitution derivatives of cellulose soluble in organic solvents, by subjecting them to the action of hot aqueous media, and subsequently esterifying the materials of reduced luster, the structure of the 45 materials being maintained during the esterification process.

2. Process for the production of artificial materials of reduced luster which is not increased by ironing while wet, which comprises acetylating 50 textile materials, foils, films and similar materials made of acetone-soluble cellulose acetate, the luster of which has been reduced by hot aqueous media, by subjecting them to treatment in a liquid non-solvent acetylation medium comprising acetic anhydride dissolved in a non-solvent diluent in the presence of ferric chloride as catalyst.

3. Process for the production of artificial ma-

terials of reduced luster which is not increased by ironing while wet, which comprises acetylating textile materials, foils, films and similar materials made of acetone-soluble cellulose acetate, the luster of which has been reduced by hot aqueous media, by subjecting them to treatment in a liquid non-solvent acetylation medium comprising acetic anhydride dissolved in a non-solvent diluent in the presence of stannic chloride as catalyst.

4. Process for the production of artificial materials of reduced luster which is not increased by ironing while wet, which comprises acetylating textile materials, foils, films and similar materials made of acetone-soluble cellulose acetate, the luster of which has been reduced by hot aqueous media, by subjecting them to treatment at a temperature of about 20 to 25° C. in a liquid non-solvent acetylation medium comprising acetic anhydride dissolved in a non-solvent diluent selected from the group consisting of liquid hydrocarbons and halogenated hydrocarbons in the presence of ferric chloride as catalyst, the amount of acetic anhydride being from 5 to 20% of the amount of non-solvent diluent.

5. Process for the production of artificial materials of reduced luster which is not increased by ironing while wet, which comprises reducing the luster of textile materials, foils, films and similar materials made of acetone-soluble cellulose acetate, by subjecting them to the action of hot aqueous media and subsequently acetylating the materials of reduced luster by subjecting them to treatment at a temperature of about 20 to 25° C. in a liquid non-solvent acetylation medium comprising acetic anhydride dissolved in a non-solvent diluent selected from the group consisting of liquid hydrocarbons and halogenated hydrocarbons in the presence of ferric chloride as catalyst, the amount of acetic anhydride being from 5 to 20% of the amount of non-solvent diluent.

6. Process for the production of artificial materials of reduced luster which is not increased by ironing while wet, which comprises esterifying textile materials, foils, films and similar materials made of organic substitution derivatives of cellulose soluble in organic solvents, the luster of which has been reduced by hot aqueous media, by subjecting them to treatment in a liquid non-solvent esterification medium comprising an organic acid anhydride dissolved in a non-solvent diluent in the presence of a metal halide having an acidic reaction as catalyst, the structure of the materials being maintained during the esterification process.

HENRY DREYFUS.